

## UNITED STATES PATENT OFFICE

2,397,756

## THERMOELECTRIC DEVICE

Ernst Schwarz, Enfield, England

No Drawing. Application December 24, 1942,  
Serial No. 470,032. In Great Britain July 2,  
1941

3 Claims. (CL 136—5)

This invention consists of improvements in or relating to thermo-electric devices. Many different proposals have been made for producing suitable elements for thermocouples and in particular for obtaining a high degree of sensitivity in thermopiles. It is known that to obtain a high sensitivity it is necessary that the substances used must possess a high thermo-electric power and that the loss of heat from the irradiated surface must be kept as small as possible. To minimize heat loss it has been customary to use the thermo-electric elements in the form of fine wires or strips sometimes joined end to end but these arrangements are delicate and are apt to be injured by shock or vibration. When attempts have been made to construct these fine or thin elements from metals or compounds of high thermo-electric power like metallic tellurium or bismuth or antimony or their alloys they are found to be very brittle so that they are difficult to handle and do not effectively resist shock and vibration.

One object of this invention is to provide compositions suitable for thermo-electric elements of high and variable thermo-electric power and low heat conductivity which shall be strong and tough and readily worked.

The conditions which these compositions should fulfil are that they should have the following properties:

- (1) High and reliable thermo-electric power capable of variation.
- (2) Low specific resistance.
- (3) Low heat conductivity.
- (4) Good mechanical properties.
- (5) Appropriate melting point neither too low nor too high (e. g. between 500° C. and 800° C.).
- (6) Resistance to oxidation (on heating in air).
- (7) Weldability to metals such as silver or gold.
- (8) Stability either in air or vacuum.
- (9) In certain cases, as in pyrometers, a low rate of change of resistance with temperature.

According to this invention a composition is made from a metal or from two or more metals combined with two or more elements of the sulphur group.

All the conditions mentioned above are fulfilled if the composition consists of one, two or three metals with elements of the sulphur group. The convenient metals are silver, copper, lead and thallium and the elements of the sulphur group are sulphur, selenium and tellurium.

It is to be understood that if both thermo-electric elements contain two or more metals combined with two or more elements of the sul-

phur group the thermo-electric effect is secured by arranging that in one thermo-electric composition the proportion of a certain metal or compound (or of certain metals or compounds) is comparatively high whereas in the other thermo-electric composition the proportion of the constituent metals and elements is substantially different. By alteration of the proportions it is possible to fulfil all the nine conditions set out above.

A metal such as silver may be melted with sulphur and selenium to form a composition for use as one element in a thermo-electric device. This composition may contain minor proportions of other metals such as copper or lead and/or tellurium. For example, one element herein referred to as the positive element may have a composition as follows:

|           | Per cent |
|-----------|----------|
| Copper    | 1        |
| Silver    | 78       |
| Tellurium | 0.6      |
| Selenium  | 13       |
| Sulphur   | 7.4      |

It is found that by varying the proportions of the elements in the above composition, the thermo-electric power against platinum can be varied within a range of about 130 to 1200 microvolts per degree centigrade. An increase of sulphur and reduction in selenium increases the thermo-power. Increase in tellurium decreases the specific resistance and the rate of change of resistance with temperature. Thus in producing a positive element the amount of copper is preferably less than 2%, the amount of silver may range between 70 and 80%, the amount of selenium may range between 10 and 15%, the amount of sulphur may range between 5 and 10%, and the amount of tellurium is preferably less than 2%.

Copper and silver and tellurium with selenium and sulphur are melted together to form a composition for use as another element of a thermo-electric device (say the negative element) and the following is one example of an appropriate composition, the figures being given as percentages by weight:

|           |    |
|-----------|----|
| Copper    | 27 |
| Silver    | 32 |
| Tellurium | 33 |
| Selenium  | 7  |
| Sulphur   | 1  |

In producing a negative element the amount of copper may range between 25 and 30%, the

amount of silver may range between 25 and 35%, the amount of tellurium may range between 30 and 35%, the amount of selenium may range between 5 and 10%, and the amount of sulphur is preferably less than 2%.

Certain other metals may be used in the thermo-electric compositions: thus lead in proper proportions may increase the thermo-power of said compositions and may also improve the mechanical properties by making the bodies tougher, more ductile or harder. Thallium may also be added. A simple test may be necessary to determine the appropriate proportion of such additions because their effect varies with the composition of the remainder.

These compositions are not brittle but quite tough and they can be made into suitable forms for securing, say by welding, to conducting supports and to irradiation surfaces.

The present invention can be used in conjunction with that described in my United States patent application Serial No. 470,031 filed December 24, 1942, that is to say, the two compositions may be used in the form of little sturdy bodies (say conical or cylindrical bodies) secured to the outer ends of supporting pillars of conducting material and the tips of these bodies may be secured to the back of a metallic foil the outer surface of which is the irradiation surface.

These bodies are semi-conductors of electricity and have a low heat conductivity.

The thermo-electric powers of the two bodies (in relation to gold or platinum) may be of opposite sign so that their thermo-electric effects are added when the device is in operation in a completed circuit.

It will be understood that for different types of instruments involving the use of thermo-electric couples the conditions or requirements may vary and, as has been pointed out, the thermo-electric power, the electric resistance, the thermal conductivity and the mechanical properties such as toughness and ductility vary with the constituents and their proportions. For any particular use of this invention a simple test may be necessary to determine the optimum composition for the two elements respectively.

If the two bodies were placed in contact it would be comparatively difficult to join them but it is a subsidiary feature of this invention that in

the preferred arrangement the bodies above referred to are conductively connected, say by electric welding, to the supporting pillars and to the foil or receiver.

5 This invention can be applied to the following uses:

1. In thermopiles for detecting and measuring radiation;

10 2. In thermo-converters for converting alternating to direct current;

3. In the transformation of radiation energy (say from the sun) into electric current;

15 4. For measuring degree of vacuum (as the sensitivity of the thermo-electric device increases as the gaseous pressure diminishes);

5. In electrical relays affected by radiation as in burglar alarms;

20 6. In pyrometers for measuring the total radiation from any body;

7. In differential or thermo relays.

Hitherto in making and using thermopiles difficulties have arisen due to the interconnection between the resistance and the sensitivity, because several of the conditions under which a thermopile is used (including, for example, the type of galvanometer) call for an independent selection of the resistance and sensitivity of the thermopile. It is one of the practical advantages of the present invention that the resistance and the sensitivity of the thermopile can be independently varied to an outstanding extent.

I claim:

1. A thermo-electric couple having a positive thermo-electric element comprising a fused material containing between 70 and 80% silver, less than 2% copper, 10 to 15% selenium, 5 to 10% sulfur, and less than 2% tellurium, and a negative thermo-electric element comprising a fused material containing 25 to 30% copper, 25 to 35% silver, 30 to 35% tellurium, 5 to 10% selenium, and less than 2% sulphur.

2. A positive thermo-electric element comprising a fused material containing between 70 to 80% silver, less than 2% copper, 10 to 15% selenium, 5 to 10% sulphur, and less than 2% tellurium.

3. A negative thermo-electric element comprising a fused material containing 25 to 30% copper, 25 to 35% silver, 30 to 35% tellurium, 5 to 10% selenium, and less than 2% sulphur.

ERNST SCHWARZ.